

# United States Patent [19]

Ohtani et al.

[11] 3,802,939

[45] Apr. 9, 1974

[54] SURFACE-HARDENED TITANIUM OR ZIRCONIUM AND THEIR ALLOYS AND METHOD OF PROCESSING SAME

[75] Inventors: Shitoshi Ohtani, Saita; Minoru Nishigaki, Akashi, both of Japan

[73] Assignee: Kobe Steel, Ltd., Fukiai-ku, Kobe, Japan

[22] Filed: Mar. 22, 1971

[21] Appl. No.: 126,630

[52] U.S. Cl. .... 148/133, 29/198, 148/32.5, 148/34, 148/127

[51] Int. Cl. .... C22f 1/18, B32b 15/00

[58] Field of Search .... 148/31.5, 32.5, 34, 133, 148/127; 29/198, 504; 204/37; 117/131

## [56] References Cited

### UNITED STATES PATENTS

|           |        |                      |           |
|-----------|--------|----------------------|-----------|
| 3,645,803 | 2/1972 | Huber et al. ....    | 148/127 X |
| 3,560,274 | 2/1971 | Ogden ....           | 29/198    |
| 2,940,163 | 6/1960 | Davies ....          | 29/198 X  |
| 3,493,353 | 2/1970 | Bergmann et al. .... | 29/198 X  |

2,932,887 4/1960 McCuaig et al. .... 29/198 X

## OTHER PUBLICATIONS

Metallurgio, December 1957, pages 277-282

Metal Selector, 1963 Edition - Reprinted from Oct. 14, 1963 Steel, page S-40

Primary Examiner—Charles N. Lovell

Attorney, Agent, or Firm—Oblon, Fisher, Spivak, McClelland & Maier

## [57] ABSTRACT

Surface-hardened pure titanium or pure zirconium, titanium-base alloys, or zirconium-base alloys having an aged coating of a metastable beta alloy layer of a titanium or zirconium-base metal applied thereon. A method of hardening the surface of pure titanium, pure zirconium, titanium-base alloys, or zirconium-base alloys, which includes coating a metastable beta alloy of a titanium-base or zirconium-base metal thereon, and aging said coated alloy at temperatures of 200°-600°C.

12 Claims, 2 Drawing Figures

PATENTED APR 9 1974

3,802,939

FIG. 1



FIG. 2



INVENTORS  
SHITOSHI OHTANI  
MINORU NISHIGAKI

By *Olson, Fisher & Spirak*  
ATTORNEYS

**SURFACE-HARDED TITANIUM OR  
ZIRCONIUM AND THEIR ALLOYS AND METHOD  
OF PROCESSING SAME**

**BACKGROUND OF THE INVENTION**

**1. Field Of Invention**

This invention relates to surface-hardened titanium, zirconium or their alloys and to a method of preparing same. More particularly, this invention relates to surface-hardened, pure titanium, pure zirconium, titanium-base alloys, or zirconium-base alloys, and to a method of surface-hardening such metals.

**2. Description Of The Prior Art**

Generally, titanium and zirconium have superior corrosion resistance in comparison with the other metals, and accordingly they are broadly used in the chemical field as well as many other technologies. However, since these metals have a disadvantageously low hardness, if they are frictioned with any other metal, seizures tend to occur, which greatly limits the range of possible applications for these types of metals.

It has previously been proposed to harden the surface of metals of this type such as by nitriding their surfaces. Surface nitriding utilizes the fact that titanium and zirconium are greatly activated at high temperatures above 500°C., and combine at high temperatures above 800°C. to form a solid solution of nitrides and a diffusion layer. Usually, the titanium or zirconium is contact-treated with a nitriding gas at temperatures of from 800°-900°C. so as to harden their surfaces. Although this method has been commercially applied, since the surface-hardened layer obtained is extremely thin, its endurance period is very short, in spite of the very complicated treating operation. Other prior art methods also have similar disadvantages, and hence are similarly ineffective for many commercial applications.

**SUMMARY OF THE INVENTION**

Accordingly, one object of the present invention is to eliminate the aforementioned disadvantages of conventional methods and to provide a novel and improved surface-hardened titanium, zirconium, or alloy thereof, and to provide a method of processing the same.

Another object of the present invention is to provide a surface-hardened pure titanium or pure zirconium.

A further object of the present invention is to provide a surface-hardened titanium-base or zirconium-base alloy.

An additional object of this invention is to provide a method of hardening the surface of pure titanium, pure zirconium, or titanium-base or zirconium-base alloys.

Briefly, these and other objects are attained in one aspect of the present invention wherein surface-hardened pure titanium or zirconium is provided by a process which comprises coating a metastable beta alloy layer of a titanium or zirconium-base metal onto said pure metal, and aging said coating to give a hardness of at least 400 Vickers hardness or above. The aforementioned metastable beta alloys may be any of the Ti(Zr)-Mo type, Ti(Zr)-V type, Ti(Zr)-Fe type, Ti(Zr)-Cr type, Ti(Zr)-Mn type, Ti(Zr)-Nb type, Ti(Zr)-Ta, and multi-element type alloys containing three or more elements of the aforesaid two-element type alloys.

According to another aspect of the present invention, surface-hardened titanium-base or zirconium-base al-

loys are provided by a process which comprises coating a metastable beta alloy layer of a titanium or zirconium-base metal onto said alloy and aging as above. The aforesaid titanium-base alloys may be of a Ti-6Al-4V type, Ti-5Al-2Cr-1Fe type, Ti-5Al-2.5Sn type, Ti-0.2Pd type, Ti-8Mn type, Ti-8Al-1Mo-1V type, Ti-6Al-6V-2Sn type, Ti-4Al-3Mo-1V type, Ti-2Cu type, Ti-2Al-2Mn type, Ti-2.25Al-11Sn-5Zr-1Mo-0.1Si type, Ti-5Al-5Sn-5Zr type, and the like.

The aforesaid zirconium-base alloys may be Zircaloy-2, Zircaloy-4, and the like.

According to a further aspect of this invention, there is provided a method of hardening the surface of pure titanium, pure zirconium, or titanium-base or zirconium-base alloys, which comprises the steps of coating a metastable beta alloy of a titanium-base or zirconium-base metal thereon and aging said coated alloy at temperatures of 200°-600°C. Thus, a surface-hardened layer may be very effectively formed on the surface of the metal to be treated according to this invention, in various thickness suitable for the intended purpose.

In the method of this invention, if the metastable beta alloy of the titanium-base or zirconium-base metal is aged at low temperatures of 200°-600°C., the beta phase is decomposed to precipitate the alpha phase or its intermediate phase, i.e., omega phase, and the alloy is extremely hardened. This fact is utilized in this invention in such a manner that the metastable beta phase alloy of this type is coated in advance on the surface of the metal to be treated, and then the coated surface is aged at a low temperature region so as to harden only the surface layer, providing a titanium or zirconium product.

The coating of the metastable beta phase alloy may be provided on the surface of the metal to be treated, for example, by diffusion welding or explosive pressure welding. The most effective and simplest method, however, will often be deposit welding. In this case, since the metastable beta phase alloy to be deposited on the metal surface to be treated is common to the metal to be treated in the base metal, the welded portion will have no possibility of becoming fragile by metallurgical reaction.

In the method of this invention, the coated surface is aged in the temperature range of 200°-600°C. for a suitable period of time in the range of 5 minutes to 20 hours. If the aging is performed for a period shorter than 5 minutes, difficulty may be experienced in industry, and use of times longer than twenty hours is not efficient for industry.

The other treating operations may be in accordance with the common conditions known by those skilled in the art.

**BRIEF DESCRIPTION OF THE DRAWINGS**

A more complete appreciation of the invention will be readily obtained as the same becomes better understood by reference to the following detailed description when taken in conjunction with the accompanying drawings, wherein:

FIGS. 1 and 2 are graphical representations of the hardness distribution obtained from a titanium-base alloy treated in accordance with the present invention.

## DETAILED DESCRIPTION OF PREFERRED EMBODIMENTS

Reference is now made to FIG. 1, which shows the hardness distribution obtained by the method of this invention. Pure titanium plate was prepared as the base metal to be treated. Ti-15Mo-5Zr type alloy was deposited by TIG welding on the surface of the pure titanium plate, which was then held in aging treatment for six hours at 450°C. Thus, as shown in FIG. 1, a surface-hardened layer having sufficiently high hardness could be obtained.

Referring now to FIG. 2, which also shows the hardness distribution obtained by the method of this invention, a titanium-base alloy plate of the Ti-5Al-2Cr-1Fe type was prepared as the base metal to be treated. This alloy was also deposited in a manner similar to the method described above with reference to FIG. 1. The deposited alloy was then subjected to solution treatment at a temperature of 800°C. for 2 hours, cooled by water, age treated at a temperature of 450°C. for 6 hours, and finally cooled by air. Thus, as shown in FIG. 2, a surface-hardened layer having sufficiently high hardness could also be obtained.

It will be understood from the foregoing description that the surface-hardened pure titanium, pure zirconium, or titanium-base or zirconium-base alloys of this invention have a coating of a metastable beta alloy layer of a titanium or zirconium-base metal which has been aged to a sufficient hardness. The thickness of the surface-hardened layer may be selected in accordance with the intended use. Furthermore, since this layer before the aging treatment is relatively soft, as seen from the graphs shown in the drawings, it is possible to easily work the metal, such as by cutting it or the like, even after the metal is coated, and thereafter age the coating to form the hardened surface. Thus, the method of this invention is particularly adapted for producing agitator blades, valves, bushings, etc.

It should also be understood that since the method of this invention forms an aged coating of a metastable beta phase alloy of the same type of metal as that to be treated, the thickness of the surface-hardened layer may be suitably selected to suit the desired product. It is also possible to work the metal to any shape, due to 45 the aforementioned effects.

It will be appreciated that, while the foregoing disclosure relates only to preferred embodiments of the invention for preparing surface-hardened pure titanium or zirconium, or titanium-base or zirconium-base alloys, numerous modifications or alterations will be apparent to those skilled in the art without departing from the spirit and scope of the invention as set forth in the appended claims.

What is claimed as new and intended to be secured by letters patent of the United States is:

1. A titanium or titanium base alloy having a deposited Ti metastable beta alloy layer thereon, said deposited layer being in an age hardened condition and having a hardness of at least 400 Vickers wherein said titanium base alloy is selected from the group consisting of Ti-6Al-4V, Ti-5Al-2Cr-1Fe, Ti-5Al-2.5Sn, Ti-0.2Pd, Ti-8Mn, Ti-8Al-Mo-1V, Ti-6Al-6V-2Sn, Ti-4Al-3Mo-1V, Ti-2Cu, Ti-2Al-2Mn, Ti-2.25Al-11Sn-5Zr-1Mo-0.1Si, and Ti-5Al-5Sn-5Zr and wherein said metastable beta alloy is selected from the group consisting of Ti-Mo, Ti-V, Ti-Fe, Ti-Cr, Ti-Mn, Ti-Nb, Ti-Ta and alloys containing three or more elements of the aforesaid two element alloys.

0.1Si, and Ti-5Al-5Sn-5Zr and wherein said metastable beta alloy is selected from the group consisting of Ti-Mo, Ti-V, Ti-Fe, Ti-Cr, Ti-Mn, Ti-Nb, Ti-Ta and alloys containing three or more elements of the aforesaid two element alloys.

2. A zirconium or zirconium base alloy having a deposited Zr metastable beta alloy layer thereon, said deposited layer being in an age hardened condition and having a hardness of at least 400 Vickers, wherein said zirconium base alloy is selected from the group consisting of zircaloy-2 and zircaloy-4 and wherein said metastable beta alloy is selected from the group consisting of Zr-Mo, Zr-V, Zr-Fe, Zr-Cr, Zr-Mn, Zr-Nb and Zr-Ta, and alloys containing three or more elements of the aforesaid two element alloys.

3. The titanium or titanium base alloy of claim 1, wherein said age hardening was conducted at a temperature of from 200° - 600°C.

4. The zirconium or zirconium base alloy of claim 2, wherein said age hardening was conducted at a temperature of from 200° - 600°C.

5. A method of hardening the surface of a titanium or titanium base alloy which comprises depositing a layer of a Ti metastable beta alloy onto the surface of said titanium or titanium base alloy, solution heat treating, quenching, and aging said alloy layer at temperatures of 200° - 600°C. for a period of 5 minutes to 20 hours to a Vickers hardness of at least 400, wherein said titanium base alloy is selected from the group consisting of Ti-6Al-4V, Ti-5Al-2Cr-1Fe, Ti-5Al-2.5Sn, Ti-0.2Pd, Ti-8Mn, Ti-8Al-Mo-1V, Ti-6Al-6V-2Sn, Ti-4Al-3Mo-1V, Ti-2Cu, Ti-2Al-2Mn, Ti-2.25Al-11Sn-5Zr-1Mo-0.1Si, and Ti-5Al-5Sn-5Zr and wherein said metastable beta alloy is selected from the group consisting of Ti-Mo, Ti-V, Ti-Fe, Ti-Cr, Ti-Mn, Ti-Nb, Ti-Ta and alloys containing three or more elements of the aforesaid two element alloys.

6. A method of hardening the surface of a zirconium or zirconium base alloy which comprises:

depositing a layer of a Zr metastable beta alloy onto the surface of said zirconium or zirconium base alloy, solution heat treating, quenching, and aging said alloy at temperatures of 200° - 600°C. for a period of 5 minutes to 20 hours to a Vickers hardness of at least 400, wherein said zirconium base alloy is selected from the group consisting of zircaloy-2 and zircaloy-4 and wherein said metastable beta alloy is selected from the group consisting of Zr-Mo, Zr-V, Zr-Fe, Zr-Cr, Zr-Mn, Zr-Nb and Zr-Ta, and alloys containing three or more elements of the aforesaid two element alloys.

7. The method of claim 6, wherein said metastable beta alloy is formed by diffusion welding.

8. The method of claim 6, wherein said metastable beta alloy is formed by explosive pressure welding.

9. The method of claim 6, wherein said metastable beta alloy is formed by deposit welding.

10. The method of claim 5, wherein said metastable beta alloy is coated by diffusion welding.

11. The method of claim 5, wherein said metastable beta alloy is formed by explosive pressure welding.

12. The method of claim 5, wherein said metastable beta alloy is formed by deposit welding.

\* \* \* \* \*